

# UNITED STATES PATENT OFFICE

AMÉDÉE J. LANFREY, OF CHARTRES, FRANCE.

## MANUFACTURE OF EXPLOSIVE COMPOUNDS.

SPECIFICATION forming part of Letters Patent No. 276,833, dated May 1, 1883.

Application filed June 9, 1879. Patented in France June 12, 1878, No. 124,769; in Belgium August 6, 1878, No. 49,833; in England August 7, 1878, No. 3,119; in Italy August 17, 1878; in Austria April 7, 1879, No. 5,521; in Portugal June 11, 1879; in Germany January 21, 1880, No. 12,119, and in Sweden August 28, 1880.

To all whom it may concern:

Be it known that I, AMÉDÉE JOSEPH LANFREY, of Chartres, in the Republic of France, and an officer in the French army, have made 5 certain new and useful Improvements in the Manufacture of Explosive Compounds, of which the following is a full, clear, and exact description.

The object of this invention is improvements in the manufacture of certain explosive compounds, the basis of these new explosive substances consisting of various straws, such as corn, rye, barley, oats, and buckwheat. It is manufactured as follows: The straw is submitted to a boiling operation for fifteen or sixteen hours in an alkaline solution (carbonate of soda or of potassium) weighing from 20 to 30 Baumé. In this state the straw easily disintegrates, and the fatty or other soluble matters which it contained are dissolved and carried off by the water when the latter is withdrawn. The fibers are then triturated, and a perfect washing effected at the same time, either by means of a cylinder stuff-engine similar to those employed in paper-mills or by means of revolving millstones, also similar to those used in such mills. During the trituration a current of water should constantly wash the fibers. It is essential that 25 this pulp does not retain any alkaline reaction, which is insured by adding sulphuric or hydrochloric acid in sufficient quantity that the washing-water has a slightly-acid reaction. The fibers thus triturated and prepared 30 are, after having been perfectly dried, ready to undergo the reactions which render them explosive. To facilitate the manipulations which follow, the pulp is treated by a paper-machine, and should produce a sheet weighing about three hundred grams the square meter. The thickness may vary more or less. The sheet thus formed is cut, either by hand 35 by the aid of special tools, or mechanically, into little pieces of three to four millimeters square. These little pieces or fragments are then immersed for three or four hours in an acid compound composed of three volumes of smoking ("fumant") azotic acid (at 46° to 48°) and seven volumes of concentrated sulphuric acid, (at 66°,) then withdrawn from the

acid bath, drained as much as possible, pressed, and finally well washed with water until there remains no trace of acid. Any acid reaction is prevented by adding to the last washing-water a little carbonate of potassium or of soda, and a little of this alkaline water is left in contact with the little pieces or fragments for several hours. The fragments may be immersed in a compound of nitrate of soda or potassium and concentrated sulphuric acid for 55 their more economic transformation into nitro-cellulose, the result being the same.

The object of making the sheets into fragments is to facilitate the action of the acids, and this result might, it is obvious, be obtained by punching holes in the sheet. In this case the acid may be pressed from the sheet by valves which are not acted upon by the acids. It is preferable to repeat the immersion in the acids and the expression of 60 the portion absorbed.

The nitro-cellulose thus obtained has peculiar properties which fit it for use as an agent for blasting or use in fire-arms independent of the quality of exploding which it has in connection with all other kinds of nitro-cellulose. 75 These properties are as follows:

First, stability and resistance to shocks, the inertia being in proportion to the contained silica. From analysis by Sprengel, oat-straw 80 is found to contain 4.59 per cent., wheat 2.87 per cent., and the other straws still somewhat less, barley being 2.86 per cent. and rye 2.30 per cent.

Second, regularity of explosion and less rapid 85 deflagration in fire-arms, due to silica.

Third, ability to obtain a weak nitrification, together with a product of homogeneous constitution, for employment in fire-arms, in which the combustion should be slow, progressive, and regular. Pure cellulose is nitrated 90 too strongly, or, if the immersion in the acid bath has been for a very short time, one part is strongly nitrated and another not at all, so that a mixture is formed of cellulose and nitro-cellulose. In other words, the constitution is not homogeneous. Straw cellulose, which may be regarded as formed of pure cellulose and silica, in consequence of the presence of the latter in intimate contact therewith, is nitrated feebly 95 100

and regularly even after a contact with the acids long enough for them to penetrate the entire mass. By "feeble nitration" is to be understood that which produces nitro-cellulose, and not trinitro-cellulose. Nitro-cellulose from straw satisfies, therefore, the condition mentioned—to wit, it is nitrated feebly, so that the combustion is slow and progressive, and is of a homogeneous constitution, which gives 10 regularity to the explosion.

Fourth, a power of absorption, which exists in a higher degree in this material than in nitro-cellulose from wood or cotton. It is well known that cellulose exists in many forms 15 from the hard shell of the seed of the plum or cherry to young sprouts, and the nitro-cellulose from these materials differs in like manner. Nitro-cellulose from straw can absorb seventy-five per cent. of nitro-glycerine, which 20 is not possible with ordinary gun-cotton or nitrated wood. Nitro-cellulose from straw is itself different from that obtained from bamboo or cane, and the process applicable to its manufacture could not be employed for the 25 nitration of bamboo. The composition of bamboo is different from straw, and their nitrated products differ in like manner. The capacity for separation, consistency, and absorbing power is entirely different. The cellulose in 30 cane and bamboo resembles that of wood more than straw, their rigidity being due to a large quantity of incrustating material called "lig-nine," (a matter which is very difficult to remove,) and not to the presence of silica, which 35 is contained in very small quantity. Moreover, straw is an article found universally in civilized nations, while bamboo is only encountered over limited areas. The production of nitro-cellulose from straw is also more economical 40 than from other materials, such as cotton, flax, bamboo, or the like.

Having thus explained the special properties of straw nitro-cellulose, the description of the process is continued as follows:

45 Nitro-cellulose prepared according to this invention has been kept for upward of three years without suffering any deterioration nor

losing any of its explosive force, nor has any accident occurred resulting from spontaneous ignition during the numerous experiments to 70 which it has been subjected. The cause of this stability (of such great importance in explosive bodies) is the following: The straw fibers are formed of cellulose containing, when in a combined state, a considerable quantity of silica 75 in the form of silicates. This silica in straw nitro-cellulose plays a part analogous to that which it fulfills in dynamite, in which it fixes the nitro-glycerine and imparts an amount of stability to that substance which it does not 80 possess when alone. For this reason preference is given to wheat-straw for the present process in consequence of its containing more silica than other straws, although they may, however, produce good results. 85

The novelty of the chemical reaction of the azotic acid on vegetable fibers is not claimed, as this has been known more than thirty years; but what is claimed is the novelty of the product obtained from a disintegrated and purified 90 raw material which has never before been availed of for this purpose. This production is not gun-paper, because the straw fibers purified as above described would produce exactly the same explosive without being previously transformed into paper, which is only to facilitate the subsequent operations. Considerable economy resulting from the employment of this raw material is another advantage which is claimed for this invention. These pieces of 100 straw nitro-cellulose thus neutralized, but retaining a slight alkaline reaction, are placed, after having been drained, into a solution of niter containing dextrine, and sometimes powdered charcoal, in a state of suspension in the 105 liquid.

The solutions, which are also claimed as part of the invention, vary according to the uses for which the explosives are required.

The following is a table of the average proportions of the substances which they should contain for obtaining explosive products with a basis of straw nitro-cellulose, and having various properties:

|    | Solution of niter                | At 6° to 7° Baumé's aerometer. | Rock or hard stone.                | 115 |
|----|----------------------------------|--------------------------------|------------------------------------|-----|
| 50 | Explosive for blasting purposes. | 100 Hard-wood charcoal.        | At 6° to 7° Baumé's aerometer.     |     |
|    |                                  | 25 Dextrine                    | Soft stone and earth.              |     |
|    |                                  | 100 Niter                      | 100 At 6° to 7° Baumé's aerometer. |     |
|    |                                  | 35 Hard-wood charcoal.         | Wood.                              |     |
|    |                                  | 100 Niter                      | 100                                |     |
|    |                                  | 15 Hard-wood charcoal.         | At 8° to 9° Baumé.                 | 120 |
|    |                                  | 15 Dextrine                    | Explosive for sporting purposes.   |     |
|    |                                  | 100 Niter                      | 100                                |     |
|    |                                  | 20 Hard-wood charcoal.         | At 12° to 14° Baumé.               |     |
|    |                                  | 10 Dextrine                    | Explosive for rifles.              |     |
|    |                                  | 100 Niter                      | 100                                |     |
|    |                                  | 20 Hard-wood charcoal.         | At 16° to 17° Baumé.               | 125 |
|    |                                  | 10 Dextrine                    | Explosive for cannon or ordnance.  |     |

60 The little pieces are steeped for at least an hour in the solution chosen, care being taken to stir up the mixture at intervals, after which they are drained off and perfectly dried by means similar to those employed to dry ordinary gunpowder.

65 It has been ascertained by numerous experiments that blasting force and shooting force

of this substance, compared with ordinary gunpowder, is as three to one.

An exceedingly energetic dynamite which may be obtained by the compound of straw nitro-cellulose with nitro-glycerine is also claimed. It is formed as follows: The nitro-cellulose is crushed in contact with two per cent. of carbonate of soda or of potassium un-

der the action of revolving millstones or of stampers. In this operation the nitro-cellulose must contain twenty to thirty per cent. of moisture. The operation is continued until the mass 5 appears to be nearly reduced to a powder, after which the mixture with nitro-glycerine may be made either by drying the nitro-cellulose or mixing them in a moist state and afterward dried. The proportions of nitro-glycerine to be introduced vary according to the use for which they are required. They may be from one to seventy-five per cent. In the proportion of fifty per cent., any exudation is impossible under a great pressure, and the 10 force of this dynamite is very considerable, as may be seen by the following figures, compared with those of dynamite having an inert basis, and with pure nitro-glycerine: Two grams of explosive substance placed in holes 0.01 15 meter in diameter by 0.08 meter long in cylindrical blocks of lead and filled up with water produced, by Nobel's No. 1 dynamite, containing seventy-five per cent. of nitro-glycerine; straw dynamite, or "paleine," containing fifty 20 percent of nitro-glycerine; pure nitro-glycerine. Ten to fifteen per cent. of saltpeter may be added to the nitro-cellulose by way of economy; but the explosive force is not increased thereby, the oxygen in excess of the nitro-glycerine 25 being sufficient to combine all the free carbon of the nitro-cellulose. This combination explains the large quantity of gas produced by straw dynamite or paleine.

The advantages of this compound over gun-cotton dynamites are, first, a greater physical 30 stability, inertia, resistance to the mechanical action of concussions or detonating bodies by reason of the silicate in combination in the straw, consequently greater safety in its employment; secondly, considerable economy.

This straw dynamite or paleine, like gun-cotton dynamite, does not freeze, and easily explodes at a very low temperature. It always retains its plasticity.

Explosives of various compositions may be 45 manufactured by varying the proportions of the substances employed.

Having now described the nature of the said invention and in what manner the same is to be performed, I declare that I claim— 50

1. The improved process of manufacturing nitro-cellulose by means of straw disintegrated, triturated, washed, treated with acid, and then washed and disacclimated, as before described. 55

2. The process of manufacturing nitro-cellulose from straw, consisting in disintegrating and otherwise preparing the straw fiber, as before set forth, forming sheets or leaves from said fiber, and then treating the paper or leaves 60 with acids to convert the cellulose into nitro-cellulose, substantially as described.

3. Nitro-cellulose from straw, substantially as described, the same being in the form of paper or in other suitable form, substantially 65 as described.

4. An explosive composition for blasting or shooting purposes, consisting of nitro-cellulose from straw and explosive or oxidizing substances, as specified, such as nitro-glycerine, 70 niter, or mixtures of niter and carbonaceous matter, as set forth.

In testimony whereof I have signed my name to this specification before two subscribing witnesses.

A. LANFREY.

Witnesses:

L. RENARD,  
CHARLES MARDELET.